

Jan. 27, 1942.

C. H. BOYS

2,271,474

## SHOE FINDING

Filed June 15, 1940



Clyde H. Boys

INVENTOR.

BY Cleveland B. Hellabaugh

## UNITED STATES PATENT OFFICE

2,271,474

## SHOE FINDING

Clyde H. Boys, Drexel Hill, Pa., assignor to  
 Hercules Powder Company, Wilmington, Del.,  
 a corporation of Delaware

Application June 15, 1940, Serial No. 340,639

10 Claims. (CL. 36—77)

This invention relates to impregnated absorptive materials and more particularly to improved impregnated box toes and/or counter stiffeners for shoes, boots, and the like.

Box toes and/or counter stiffeners for shoes, boots, or the like, usually comprise a base of absorptive material, for example, felt, which is impregnated with a composition adapted to stiffen the material and render it suitable for use as a reinforcing member. The present invention 10 aims to provide box toes and/or counter stiffeners which are impregnated with a composition of this type, whereby the box toe and/or counter construction is greatly improved.

An object of the present invention is to provide box toes and/or counter stiffeners which are strong and somewhat pliable.

Another object is to provide a box toe and/or counter stiffener impregnated with a composition which is highly resistant to oxidation and decomposition.

Another object is to provide a composition which will not be attacked by perspiration and is resistant to rotting or softening.

Another object is to provide a composition which is odorless and will not have any irritating effects upon the feet.

A further object is to provide a composition which is readily prepared and applied to materials suitable for box toes and/or counter stiffeners.

Other and further objects will be obvious upon an understanding of the illustrative embodiment about to be described, or will be indicated in the appended claims, and various advantages not referred to herein will occur to one skilled in the art upon employment of the invention in practice.

In accordance with the invention, these objects may be accomplished by impregnating absorptive material such as felt, with a composition of rubber, and a hydrogenated rosin material, and a plasticizer if desired. This composition gives the foregoing results and is suitable for impregnating box toe and/or counter stiffeners for shoes, boots or the like.

In the drawing, the figure is a longitudinal sectional view of a shoe, illustrating an embodiment of the invention.

Referring to the drawing, there is shown a shoe 10 having a sole 11 and a heel 12 to which is secured the upper stock 14, lined with a suitable material 15. The shoe is provided with the usual toe construction 16 and counter construction 17, which is located at the rear end of the 55

shoe. The toe is reinforced with a box toe stiffener 19 and the counter portion is reinforced with a counter stiffener 20, both of which are located in between the upper stock 14 and the lining 15. The box toe stiffener and the counter stiffener referred to herein and in the claims as stiffening members, preferably are formed of suitable felt, impregnated with the stiffening composition about to be described.

The rosin materials which may be used in the composition are hydrogenated rosin, preferably at least 50% hydrogenated, or the glycerol, glycol, diethylene glycol, propylene glycol, trimethylene glycol, butylene glycol, pentaerythritol, mannitol, sorbitol, or the like, esters of hydrogenated rosin. The amount of hydrogenated rosin materials may be varied from about 65% to about 98% depending upon the rosin materials used, the plasticizer, if required, and the type of product desired. Preferably between about 75 and 90% of hydrogenated rosin materials is used in the composition to attain the characteristics desirable for impregnating box toe stiffeners and/or counter stiffeners and the like.

Any suitable kinds of rubber or rubber-like materials, such as Neoprene, (polymerized chlorobuta-diene), low viscosity type Vistanex (polyisobutene), or Thiokol (alkyl polysulfide condensate product), may be used in the composition, all of which will be referred to herein and in the claims as rubber or rubber materials. Preferably crepe rubber is employed because it is readily and economically rendered compatible with the hydrogenated rosin materials and provides a composition which is non-tacky and has the desired resilience, stiffness, and resistance to deterioration required to accomplish the objects of the invention.

If a plasticizer is desired to be used in the 40 composition of hydrogenated rosin material and rubber, hydrogenated methyl abietate, pine oil foots, linseed oil, China-wood oil, paraffin oil, cottonseed oil, rosin oil, castor oil, polyterpenes, and high melting point terpene ethers and esters 45 may be added in amounts varying between about one and three per cent.

The composition may be prepared by a method which generally comprises melting the hydrogenated rosin material and adding the rubber or rubber-like material thereto and the plasticizer if desired, and stirring the mass while heating at a temperature between about 250° and 270° C. for a period of between about one-half and two hours. This provides a suitable hot melt for impregnating the absorptive material.

The stiffening members are impregnated by immersing the absorptive material, such as felt, in the hot melt for about one minute and then passing the felt between a pair of rolls or other suitable devices adapted to apply slight pressure to the felt, and remove the excess melt. The felt thereafter is allowed to cool and when cooled, is tough and somewhat flexible. The felt may then be cut and formed into box toe and/or counter stiffeners.

The following examples illustrate compositions for impregnating box toes and/or counter stiffeners and the like, to accomplish the objects of the invention.

*Example 1*

|                    | Parts by weight |
|--------------------|-----------------|
| Hydrogenated rosin | 90              |
| Rubber             | 8               |
| Paraffin oil       | 2               |

Ninety parts by weight of hydrogenated rosin, and two parts by weight of paraffin oil and eight parts by weight of rubber were stirred together at 260° C. for one and one-quarter hours. The hot product was poured into a mold and allowed to cool. A hard, tough, somewhat flexible product was obtained, which was found suitable for impregnating felt used for box toe and/or counter stiffeners.

*Example 2*

|                    | Parts by weight |
|--------------------|-----------------|
| Hydrogenated rosin | 90              |
| Crepe rubber       | 8               |
| Castor oil         | 2               |

Ninety parts by weight of hydrogenated rosin, and two parts by weight of castor oil, and eight parts by weight of crepe rubber were stirred together at 265° C. for three-quarters of an hour. The product obtained was hard, tough and somewhat flexible, and was suitable for impregnating the felt.

*Example 3*

|                    | Parts by weight |
|--------------------|-----------------|
| Hydrogenated rosin | 90              |
| Crepe rubber       | 10              |

Ninety parts by weight of hydrogenated rosin and ten parts by weight of rubber was stirred together at 265° C. for one hour. The resulting product was hard, tough, somewhat flexible and suitable for impregnating the felt.

*Example 4*

|                                      | Parts by weight |
|--------------------------------------|-----------------|
| Glycerol ester of hydrogenated rosin | 90              |
| Paraffin oil                         | 3               |
| Crepe rubber                         | 7               |

Ninety parts by weight of glycerol ester of hydrogenated rosin, three parts by weight of paraffin oil, and seven parts by weight of crepe rubber were stirred together at 255° C. for one hour. The product formed was hard, tough, flexible and possessed the desirable characteristics for impregnating box toe and/or counter stiffening materials.

*Example 5*

|                                             | Parts by weight |
|---------------------------------------------|-----------------|
| Pentaerythritol ester of hydrogenated rosin | 75              |
| Crepe rubber                                | 25              |

Seventy-five parts by weight of pentaerythritol ester of hydrogenated rosin and twenty-five parts by weight of crepe rubber were stirred together

at 265° C. for one and three-quarter hours. A hard, tough, and somewhat flexible product was obtained.

*Example 6*

|                                      | Parts by weight |
|--------------------------------------|-----------------|
| Sorbitol ester of hydrogenated rosin | 90              |
| Crepe rubber                         | 10              |

Ninety parts by weight of sorbitol ester of hydrogenated rosin and ten parts by weight of crepe rubber were stirred together at 265° C. for three-quarters of an hour. The product was hard, tough, and flexible and suitable for impregnating the box toe and/or counter stiffeners felt.

From the foregoing description and examples, it will be seen that the present invention provides box toes and/or counter stiffeners which are readily and economically prepared. The stiffeners are strong, whereby they serve to reinforce the portion of the shoes at which they are located, and are somewhat flexible whereby they do not adversely affect the comfort of the wearer. The compositions with which the stiffeners are impregnated are odorless, and will not irritate the feet. They are resistant to perspiration, and will not soften on aging. The hydrogenated rosin inhibits the composition against oxidation and embrittlement.

It will be understood that the details and examples hereinbefore set forth are illustrative only and that the invention as broadly described and claimed is in no way limited thereby.

What I claim and desire to protect by Letters Patent is:

1. A stiffening member for shoes comprising an absorptive base, impregnated with a composition including a material selected from the group consisting of natural and synthetic rubbers, and a material selected from the group consisting of hydrogenated rosin and hydrogenated rosin esters.

2. A stiffening member for shoes comprising an absorptive base, impregnated with a composition including a material selected from the group consisting of natural and synthetic rubbers, and a material selected from the group consisting of hydrogenated rosin and hydrogenated rosin esters, and a plasticizer.

3. A stiffening member for shoes comprising an absorptive base, impregnated with a composition including a material selected from the group consisting of natural and synthetic rubbers, and a hydrogenated rosin material.

4. A stiffening member for shoes comprising an absorptive base, impregnated with a composition including a material selected from the group consisting of natural and synthetic rubbers, and a hydrogenated rosin material and a plasticizer.

5. A stiffening member for shoes comprising an absorptive base, impregnated with a composition consisting of a material selected from the group consisting of natural and synthetic rubbers, and hydrogenated rosin.

6. A stiffening member for shoes comprising an absorptive base, impregnated with a composition consisting of a material selected from the group consisting of natural and synthetic rubbers, hydrogenated rosin, and a plasticizer.

7. A stiffening member for shoes comprising a felt base impregnated with a composition including about 90 parts by weight of hydrogenated rosin, about 8 parts by weight of crepe rubber, and about 2 parts by weight of plasticizer.

8. A stiffening member for shoes comprising an

absorptive base impregnated with a composition consisting of a material selected from the group consisting of natural and synthetic rubbers, and a hydrogenated rosin ester.

9. A stiffening member for shoes comprising an absorptive base impregnated with a composition consisting of a material selected from the group consisting of natural and synthetic rubbers, a hydrogenated rosin ester and a plasticizer. 5

10. A stiffening member for shoes comprising a felt base impregnated with a composition including about 90 parts by weight of a hydrogenated rosin ester, about 7 parts by weight of crepe rubber, and about 3 parts by weight of plasticizer.

CLYDE H. BOYS.